

March 31, 1936.

K. HAASE ET AL

2,035,804

MANUFACTURE OF POTASSIUM NITRATE

Filed July 22, 1932

Flow Table



Inventors:

Karl Haase.  
Julius Werth

## UNITED STATES PATENT OFFICE

2,035,804

## MANUFACTURE OF POTASSIUM NITRATE

Karl Haase and Hellmut Werth, Bleicherode on  
Hartz, Germany, assignors, by mesne assign-  
ments, to the firm: Preussische Bergwerks- und  
Hütten Aktiengesellschaft, Berlin, Germany

Application July 22, 1932, Serial No. 624,140  
In Germany June 15, 1932

15 Claims. (Cl. 23—102)

This invention has reference to the manu-  
facture of potassium nitrate from crude potas-  
sium salts, such as for instance from the  
so-called sylvinite or from suitable artificial or  
otherwise obtained salt mixtures by the nitration  
thereof and by conversion in aqueous solu-  
tion. In an exemplification of the principles of  
the invention we may for instance preferably  
proceed by carrying out the nitration of the  
5 crude potassium salts, such as sylvinite and  
similar salt mixtures, to the desired degree by  
means of nitrous gases obtained in the combus-  
tion of ammonia, this nitrating process being  
for instance performed with the dry salt, where-  
10 upon the nitrated salt in the second stage of  
the new process is treated with such salt solu-  
tions as will allow of converting practically all  
of the nitrates obtained into potassium nitrate.  
After the separation of the solid potassium  
15 nitrate the salt liquor may be used over again  
in the same cycle of operations for the conversion  
of new quantities of nitrated crude salts. By  
means of this method of procedure it becomes  
possible to manufacture potassium nitrate  
20 directly from two comparatively cheap raw prod-  
ucts, that is to say from crude potassium salts  
and from the gases of combustion of the oxida-  
tion of ammonia, in a short time and in a con-  
tinuous highly economical and mechanically  
25 simple manner.

In accordance with the previous state of the  
art, finished manufacturing products have been  
employed as the starting material exclusively  
or in part, and this was the main cause for the  
30 high costs and the difficulties of manufacture of  
this valuable fertilizing substance which has to  
be produced by mass-manufacturing means.  
This drawback is shared by all methods which  
make use of nitric acid or of nitrates obtained  
35 from nitric acid as the origin of nitrogen, such  
as for instance nitrate of sodium, nitrate of  
magnesium, aluminium nitrate and the like,  
while the potassium basis is obtained from  
chloride or sulfate of potassium.

40 With the employment of liquid nitric acid these  
methods present the additional difficulty of ne-  
cessitating a number of pieces of apparatus, the  
costs and operation of which are highly expensive  
and out of all proportion with the general price  
45 of commodities; besides, such kinds of appa-  
ratus, in spite of their being protected by acid-  
proof material, are subject to a very substantial  
heavy wear. For the purpose of cheapening and  
simplifying the manufacture of potassium  
50 nitrate it has already been suggested to employ

at least one of the components from which  
potassium nitrate is obtained on a large scale  
in the form of incomplete or raw manufacturing  
products. Thus, it has already been attempted  
for instance to utilize the mutual reaction of 5  
potassium crude salts with sodium nitrate in  
aqueous solution; but, even with this sugges-  
tion there is the drawback that a finished manu-  
facturing product is necessitated which must  
either be bought abroad or must be manufac- 10  
tured synthetically by means of nitric acid. It  
has also been suggested heretofore to replace  
the nitric acid by the intermediate product of  
the manufacture of nitric acid, that is to say,  
to utilize the nitrous gases for this purpose and 15  
to thus obtain potassium nitrate in the solid  
and dry condition by causing oxides of nitrogen  
to act upon potassium chloride. With this  
method, however, it was not possible to employ  
the crude potassium salts directly owing to the 20  
want of suitable direct processes of extraction  
and conversion, so that in this case also a  
finished manufacturing product had to be used  
as the potassium base. With this method there  
was the additional inconvenience that, with the 25  
use of potassium chloride the reaction with  
oxides of nitrogen proceeded very slowly so  
that the conversion into potassium nitrate was  
finished only after several days' treatment, so  
that this mode of manufacture was highly 30  
uneconomical and unsatisfactory.

In order to make our invention more clear, we  
refer to the accompanying drawing on which a  
"flow-table" is shown which will be dealt with in  
detail hereinafter. Prior, thereto, however, cer- 35  
tain statements and explanations are necessary,  
as follows:

Now the process of this invention is dis-  
tinguished from this state of the art by the  
fact that it utilizes exclusively such kinds of 40  
starting material which constitute cheap raw  
products and the conversion thereof into potas-  
sium nitrate makes it possible to dispense with  
the necessity of employing the finished pre-  
liminary manufacturing products referred to; 45  
and there is the additional advantage that it  
makes use of an operating method which allows  
of the manufacture of potassium nitrate in  
simple, inexpensive pieces of apparatus which  
are subject to a very low degree of wear only. 50  
In practising this method of manufacture it  
has been ascertained that by the employment  
of raw potassium salts in the place of potassium  
chloride and by the subdivision of the process  
of production into two stages, of which one is 55

constituted by the dry nitrating stage, while the other stage comprises a dissolving stage carried out in aqueous liquid, it becomes possible to carry out the manufacture of high-grade 5 potassium nitrate with good yields of potassium and nitrogen in a considerably shorter period of time than it has been possible with the processes heretofore in use.

Thus, it has been ascertained that, while the 10 manufacture of potassium nitrate according to the well-known processes using potassium chloride even with the use of nitrous gases took five to six days as a result of the retardation of the reaction, particularly towards the end of the 15 re-action procedure, the manufacture of this valuable fertilizer in accordance with the process of this invention is reduced to but a fraction of the period otherwise required. In accordance with this invention the favorable results and the 20 reduction of the working period are moreover assisted by the only partial nitration of the chloride compounds of the crude potassium salt (100 parts by weight of crude salt contain, for instance, 25 parts by weight of KCl, 20 to 25 25 parts by weight of  $\text{CaSO}_4$ , 50 to 55 parts by weight of NaCl) with the aid of the utilization of the higher conversion speed at the commencement of every reaction in the first section of the process (nitration) and by further treatment of the thus prepared product on an aqueous way with a certain definite assistance of the reaction by a supply of heat in the second section of the process (conversion).

The entire process of nitration of the crude 30 potassium salt according to this invention, using for instance a salt with a content of 22 to 23 percent of potassium chloride, is ordinarily terminated after about 10 hours and may even be reduced to 6 hours, if required, by the 35 use of pure dioxide of nitrogen, while the succeeding, continuously operated dissolving or conversion stage may also be carried out in a few hours.

In the first stage of the process ground crude 40 potassium salt, as for instance ground sylvinite, which may even contain small amounts of carnallite is treated in this state or in the agglomerated condition with nitrous gases, such as are formed by the combustion of ammonia, at temperatures above 100° C. This treatment may for 45 instance be effected in a furnace provided with indirectly heatable false bottoms of the type of the so-called Herreshoff-furnaces, as for instance in a scooping drier or steam-plate drier used in plants for the preparation of combustible coal or the like. In such a kind of furnace the nitration may be effected in a continuous process, the crude salt and the oxides of nitrogen being preferably caused to move in the 50 counter-current direction. The chlorides contained in the crude salt are thereby converted into nitrates, liberating chlorine which latter combines with the excess of oxides of nitrogen to form nitrosyl-chloride. It is immaterial for 55 the success of the process of this invention which of the existing chlorides of the salt are converted into nitrates, and it is moreover of no importance which of the existing chlorides is to be converted into nitrate and it is likewise of no 60 importance whether the one or the other is more or less nitrated, provided that the entire absorption of nitrogen in the form of  $\text{NO}_3$  is at least equivalent to the amount of potassium chloride originally present. Preferably, the 65 operation is carried out in such a manner that the 70 75

crude salt at the termination of the treatment contains a somewhat larger amount of nitrate than would correspond to the original contents of KCl. This small excess of nitrate may for instance be eliminated at the end of the nitrating process by the admixture of the nitrated product with non-nitrated crude salt, and in this manner the equi-molecular proportion  $\text{K}^+ : \text{NO}_3^- = 1 : 1$  required for the subsequent conversion may be obtained. The nitrosyl-chloride 10 obtained may be treated by well-known methods for the recovery of the oxide of nitrogen.

In the second stage of the process according to this invention the nitrated crude salt is treated with a suitable preheated salt solution 15 in any suitable dissolving apparatus, using for instance those kinds of dissolving apparatus which are used in the potassium-industry. The nitrates formed in the nitrating stage are thereby dissolved and converted into  $\text{KNO}_3$ . In the 20 practice of this invention the composition and the quantity of the salt solution are so adjusted that a solution is obtained which is saturated as regards  $\text{KNO}_3$ , KCl and NaCl and which may be easily separated from the undissolved admixtures. Counter to the usual expectations it has been ascertained in this connection that heating of the solution above certain temperatures for the purpose of conversion and for obtaining a potassium-nitrate of about 96% is not necessary, 25 inasmuch as even with temperatures of 50 to 70° C. for instance and in special, particularly investigated cases at 60° C., the reaction is going on with sufficient rapidity and the conditions are particularly favorable for the separation of 30 the solid admixtures. The process according to this invention presents therefore the additional advantage of a very considerable economy of heat, as compared with known methods in which the conversion of crude salt and the like is carried out at an increased temperature.

The further procedure of the second stage of the process is simple. After the separation of the residue which contains mostly NaCl and  $\text{CaSO}_4$  the hot solution which contains the entire amount of the potassium, introduced with the crude salt and the entire amount of the nitrogen of the nitrate in the form of  $\text{KNO}_3$  is mixed with a quantity of water corresponding to that amount which is lost in the residue by adhering liquid and by evaporation and is cooled. This results in the precipitation of a high-grade kind of potassium-nitrate, and a mother-liquor is obtained, the composition and quantity of which corresponds to the original 45 salt solution and which may be used again as a solvent liquid, so as to constitute a cycle of the utilization of the mother-liquor. Preferably, the operation is carried out in counter-current 50 direction. Whenever required, this potassium 55 nitrate obtained according to this invention may be treated in the well-known manner by lixiviation with some water so as to obtain absolutely pure  $\text{KNO}_3$ .

In the following we describe the above-mentioned "flow-sheet", on which the substances playing parts in the entire process are arranged, and follow one another, like a cycle, indicated in this case by quadrangles representing said substances and by connecting lines indicating their 60 flow. The details are as follows: Oxygen (quadrangle a) and ammonia (quadrangle b) are burned together in any of the known apparatus usually employed for this purpose. There arise 65 nitrous gases (quadrangle c) which are caused 70 75

to act upon sylvinite potassium crude salt (quadrangle *d*) in any of the furnaces mentioned in the preceding part of this specification. The product of this phase of the process is nitrated potassium crude salt (quadrangle *e*) which, after having been removed from the reaction apparatus employed for carrying out this phase, is continually conducted into the dissolving apparatus likewise mentioned by way of example in the preceding part of this specification, in which apparatus said nitrated potassium crude salt is treated in counter-current with pre-heated mother-lye (quadrangle *f*), the mixture being stirred during this treatment. There is obtained a hot solution (quadrangle *g*) which has taken up the nitrated portions of said crude salt, or has converted it into  $\text{KNO}_3$ , and besides this compound is obtained a residue formed by unchanged, insoluble crude salt (quadrangle *h*). This residue is separated from said hot solution by suitable means whereafter the solution is cooled, in consequence whereof potassium nitrate precipitates. This is the final product, the substance intended, that is to be turned into account. The remaining liquid constitutes the mother-lye that then is heated in a suitable apparatus and is conducted to the already mentioned mother-lye (quadrangle *f*), the lye mixture being then again used in connection with the nitrated potassium crude salt so as to deliver again a hot solution and a residue, as described. The aqueous salt solution circulates, therefore, continuously through the phases *f* and *g*, constituting circulating mother lye in the phase *f* and an aqueous hot salt solution in the phase *g*.

It should be pointed out that it could not be expected that by the use of crude salt of potassium and the like as a starting material, though it contains foreign substances, the nitration could be carried out on the dry way and in a highly satisfactory manner, and that an available product for the manufacture of potassium nitrate could be obtained by an aqueous liquid inasmuch as it was the general opinion that, for the purpose of accomplishing this result, it was necessary to employ exclusively a sufficiently pure starting material, such as manufactured by the potassium industry in the form of potassium chloride and potassium sulfate. Nor was it to be anticipated that the nitrated crude salt would yield potassium nitrate of sufficient purity by the solution and conversion of the nitrates obtained in the nitrating stage and at a dissolving temperature of for instance 60° C., nor that the converting or finishing solution could be used in a cycle of operations for the manufacture of new quantities of nitrate without any reduction of volume by evaporation and without the elimination of constituent parts of the mother-liquor. It is, moreover, an unexpected result that the time-consuming complete nitration of chloride of potassium could be replaced by a dry and merely partial nitration of the chlorides of the crude salt with the subsequent treatment by an aqueous solution at a great economy of costs and operating time.

*Experimental Example 1.*—68 grams of most finely ground sylvinite with 22% of potassium chloride are treated for 10 hours at 150° C. with a current of nitrous gases, such as are obtained in the combustion of ammonia. The yield was 73 grams of a neutral dry salt mixture containing 10.83% of potassium and 3.968% of nitrogen in the form of different nitrates. The product which contains potassium and nitrogen in the

molecular proportion of 1:1.02 was mixed with non-nitrated sylvinite or with potassium-chloride so as to present equimolecular quantities and was then treated in accordance with Example 3 described hereinafter, and worked into potassium-nitrate. The nitrosyl-chloride evolved upon the nitration of the crude salt can be recovered and worked into oxides of nitrogen in the well-known manner.

*Example 2.*—68 grams of most finely ground sylvinite with 22.8% of potassium chloride were treated for 6 hours at 150° C., and in accordance with the Example 1 with a current of pure concentrated dioxide of nitrogen. A yield of 73 grams of a salt mixture with 11.09% of potassium and 3.973% of nitrogen as nitrate was obtained. The product which contains potassium and the nitrogen of the nitrate in the molecular proportion 1:1 may be worked into potassium nitrate in accordance with Example 3 now being described.

*Example 3.*—1362 grams of sylvinite that has been nitrated in accordance with Example 1 or Example 2 and containing molecularly equal quantities of potassium and of nitrogen with 12.03% of potassium and 4.309% of nitrate-nitrogen are stirred a short time into one liter of a salt solution of the specific gravity 1.33 which contains in one liter approximately: 188 grams of  $\text{KNO}_3$ , 81 grams of  $\text{NaNO}_3$ , 148 grams of  $\text{NaCl}$ , 111 grams of  $\text{MgCl}_2$ , and 10 grams of  $\text{CaSO}_4$ , at about 60° C. The hot solution obtained was separated from the residue and cooled to 20° C., with the addition of about 99 cc. of water. The precipitated potassium-nitrate was filtered off and dried. The yield amounted to 428 grams of potassium nitrate of 96% and one liter of a salt solution of the composition above stated which could be used over again for the purpose of conversion.

It should be noted that our invention is not to be restricted to certain details of treatment and to a certain nature and proportions of materials heretofore referred to merely by way of exemplification and illustration of the principles of the invention, this latter being susceptible of modifications and variations both in the nature and in the proportions of material employed and in the mode of treatment, no other limitations being warranted and intended, except those which appear from the claims hereunto appended.

We claim:

1. The process of manufacturing potassium nitrate, comprising subjecting crude potassium salt in a dry way and at a temperature of more than 100° C. to a partial nitration with nitrous gases obtained in known manner; interrupting the nitration of said salt at a point of time at which the entire absorption of nitrogen in the form of  $\text{NO}_2$  is at least equivalent to the amount of potassium chloride originally present; treating the reaction product with an aqueous salt solution containing nitrate ions; and separating the potassium nitrate thereby formed by crystallization, substantially as set forth.

2. The process of manufacturing potassium nitrate, comprising subjecting crude potassium salt in a dry way and at a temperature of more than 100° C. to a partial nitration with nitrous gases obtained in known manner; interrupting the nitration of said salt at a point of time at which the entire absorption of nitrogen in the form of  $\text{NO}_2$  is at least equivalent to the amount of potassium chloride originally present; treat-

ing the reaction product in known manner with mother liquor obtained from a preceding cycle of similar phases of operation, and separating the potassium nitrate thereby formed by crystallization.

5 3. The process of manufacturing potassium nitrate, comprising subjecting crude potassium salt in a dry way and at a temperature of more than 100° C. to a partial nitration with nitrous 10 gases obtained in known manner; interrupting the nitration of said salt at a point of time at which the entire absorption of nitrogen in the form of  $\text{NO}_3$  is at least equivalent to the amount of potassium chloride originally present; treating 15 the reaction product in known manner with mother liquor obtained from a preceding cycle of similar phases of operation; separating from the solution in known manner the undissolved residual substances, and cooling the remaining 20 solution so as to obtain the potassium nitrate in crystalline form.

4. The process of manufacturing potassium nitrate, which comprises submitting crude salt minerals containing potassium salts to a partial 25 nitration so as to cause the conversion of the  $\text{KCl}$  to  $\text{KNO}_3$  without material conversion of the other chloride in the salt and subsequently treating the reaction product with an aqueous mixture containing water-soluble alkali salts of 30 sufficient concentration; separating and cooling the solution of the potassium nitrate, and causing the said nitrate to become separated and crystallized therefrom, and finally treating new 35 quantities of nitrated salt minerals with the mother-liquor obtained.

5. The process of manufacturing potassium nitrate with the aid of a mother lye obtained from a preceding cycle of phases of operation similar to those hereinafter stated, said method comprising submitting a solid crude salt mineral containing potassium salts to a partial substantially dry nitration to such an extent as to cause the resulting nitration product to contain potassium and the nitrate radical ( $\text{NO}_3$ ) in equi- 40 molecular quantities, and then treating said product with an aqueous salt solution identical with said mother liquor, thereby causing the base of other existing nitrates to become exchanged against the potassium base, and separating the potassium nitrate formed.

6. The process of manufacturing potassium nitrate, which comprises submitting crude salt minerals containing potassium salts to a partial nitration, interrupting the nitration of said salt 55 at a point of time at which the entire absorption of nitrogen in the form of  $\text{NO}_3$  is at least equivalent to the amount of potassium chloride originally present; treating the reaction product at an elevated temperature with an aqueous salt mixture containing nitrates of alkali and other water-soluble alkali salts; separating the solution from the residue, cooling the solution obtained, causing the potassium nitrate to precipitate, and treating new quantities of nitrated 60 mineral salts with the mother liquor.

7. A process as specified in claim 1, comprising, in combination with the phases stated in claim 1, effecting the conversion at a temperature lying between 50 and 70° C. so as to obtain 70 a solution saturated with potassium nitrate, potassium chloride, and sodium chloride; separating the residual substances from said solution, adding as much water as has been lost by 75 exhalation and as adhering solution in the re-

sidual substances, and cooling the obtained solution.

8. A process as specified in claim 1, characterized by the feature that the nitration of the starting materials is carried out only so far that the product to be nitrated contains equivalent amounts of potassium and nitrate which substances are then converted into potassium nitrate.

9. The method of producing potassium nitrate, comprising causing nitrous gases to act upon sylvinitic potassium crude salt so as to obtain nitrated potassium crude salt; treating this salt with heated mother-lye and stirring at the same time this mixture so as to obtain a hot solution that has taken up the portion of nitrate contained in said nitrated potassium crude salt, unchanged insoluble salt remaining as residue; separating said hot solution and said unchanged insoluble salt from one another, 20 cooling the said hot solution so as to cause precipitation of the potassium nitrate and to obtain at the same time mother-lye; heating this lye and conducting it back to said nitrated potassium crude salt so as to produce again a 25 hot solution of the kind stated.

10. The method of producing potassium nitrate, comprising burning ammonia with oxygen so as to obtain nitrous gases; letting these gases act upon sylvinitic potassium crude salt so as to obtain nitrated potassium crude salt; treating this salt with heated mother-lye and stirring at the same time this mixture so as to obtain a hot solution that has taken up the portion of nitrate contained in said nitrated potassium 35 crude salt; unchanged insoluble salt remaining as residue; separating said hot solution and said unchanged insoluble salt from one another, cooling the said hot solution so as to cause precipitation of the potassium nitrate and to obtain 40 at the same time mother-lye; heating this lye and conducting it back to said nitrated potassium crude salt so as to produce again a hot solution of the kind stated.

11. The method of producing potassium nitrate, comprising causing nitrous gases to act upon sylvinitic potassium crude salt so as to obtain nitrated potassium crude salt; treating this salt in counter-current with heated mother-lye and stirring at the same time this mixture 50 so as to obtain a hot solution that has taken up the portion of nitrate contained in said nitrated potassium crude salt, unchanged insoluble salt remaining as residue; separating said hot solution and said unchanged insoluble salt 55 from one another, cooling the said hot solution so as to cause precipitation of the potassium nitrate and to obtain at the same time mother-lye; heating this lye and conducting it back to said nitrated potassium crude salt so as to produce 60 again a hot solution of the kind stated.

12. The method of producing potassium nitrate, comprising causing nitrous gases to act upon sylvinitic potassium crude salt so as to obtain nitrated potassium crude salt, said gases 65 and said salt being used in such proportions relatively to one another that the entire absorption of nitrogen in the form of  $\text{NO}_3$  is at least equivalent to the amount of potassium chloride originally present; treating the nitrated potassium 70 crude salt with a heated aqueous salt solution and stirring at the same time this mixture so as to obtain a hot solution that has taken up the portion of nitrate contained in said nitrated potassium crude salt, unchanged insoluble salt 75

5 remaining as residue; separating said hot solution and said unchanged insoluble salt from one another, and cooling the said hot solution so as to cause precipitation of the potassium nitrate and to obtain at the same time aqueous salt solution.

10 13. The method of producing potassium nitrate, comprising causing nitrous gases to act upon sylvinitic potassium crude salt, said gases and said salt being used in such proportions relatively to one another that at the termination of said action the crude salt contains a somewhat larger amount of nitrate than would correspond to the original contents of KCl; 15 treating the nitrated potassium crude salt with a heated aqueous salt solution and stirring at the same time this mixture so as to obtain a hot solution that has taken up the portion of nitrate contained in said nitrated potassium 20 crude salt, unchanged insoluble salt remaining as residue; separating said hot solution and said unchanged insoluble salt from one another, and cooling the said hot solution so as to cause precipitation of the potassium nitrate and to 25 obtain at the same time aqueous salt solution.

30 14. The method of producing potassium nitrate, comprising causing nitrous gases to act upon sylvinitic potassium crude salt, said gases and said salt being used in such proportions relatively to one another that at the termination of said action the crude salt contains a somewhat larger amount of nitrate than would correspond to the original contents of KCl; admixing at the end of the nitrating phase non- 35 nitrated crude salt so as to eliminate the small excess of nitrate, the amounts being so chosen that the equimolecular proportion K:NO<sub>3</sub>=1:1

is obtained; treating the nitrated potassium crude salt with a heated aqueous salt solution and stirring at the same time this mixture so as to obtain a hot solution that has taken up the portion of nitrate contained in said nitrated potassium crude salt, unchanged insoluble salt remaining as residue; separating said hot solution and said unchanged insoluble salt from one another and cooling the said hot solution so as to cause precipitation of the potassium nitrate and to obtain at the same time aqueous salt solution. 5

15 15. The method of producing potassium nitrate, comprising, causing nitrous gases to act upon sylvinitic potassium crude salt so as to obtain nitrated potassium crude salt; treating this salt with heated mother-lye and stirring at the same time this mixture so as to obtain an aqueous hot salt solution that has taken up the portion of nitrate contained in said nitrated potassium crude salt, the amounts of the substances concerned being so chosen that said solution is saturated as regards KNO<sub>3</sub>, KCl and NaCl; separating nitrated potassium crude salt with a heated aqueous salt solution and stirring 20 at the same time this mixture so as to obtain a hot solution that has taken up the portion of nitrate contained in said nitrated potassium crude salt, unchanged insoluble salt remaining as residue; separating said hot solution and said unchanged insoluble salt from one another, and cooling the said hot solution so as to cause precipitation of the potassium nitrate and to obtain 25 at the same time aqueous salt solution. 30

35 KARL HAASE.  
HELLMUT WERTH.